

Aug. 27, 1968

E. KAUER  
INCANDESCENT LAMP WITH FILAMENT CONSISTING OF  
A HEXABORIDE OF A RARE EARTH METAL

3,399,321

Filed July 15, 1965

2 Sheets-Sheet 1



FIG.1



FIG.2

INVENTOR  
ERHARD KAUER  
BY  
*Frank R. Jifan*  
AGENT

Aug. 27, 1968

E. KAUER  
INCANDESCENT LAMP WITH FILAMENT CONSISTING OF  
A HEXABORIDE OF A RARE EARTH METAL

3,399,321

Filed July 15, 1965

2 Sheets-Sheet 2



FIG.3



FIG.4



FIG.5

INVENTOR  
ERHARD KAUER  
BY  
*Frank R. Sinfani*  
AGENT

1

3,399,321

## INCANDESCENT LAMP WITH FILAMENT CONSISTING OF A HEXABORIDE OF A RARE EARTH METAL

Erhard Kauer, Aachen, Germany, assignor to North American Philips Company, Inc., New York, N.Y., a corporation of Delaware

Filed July 15, 1965, Ser. No. 472,203

Claims priority, application Germany, July 16, 1964,

N 25,261

8 Claims. (Cl. 313—218)

### ABSTRACT OF THE DISCLOSURE

An incandescent lamp employing a filament emitting principally visible radiation at the operating temperature and consisting of a material having a concentration of charge carriers between  $2 \times 10^{21}$  and  $2 \times 10^{22}$ , the charge carriers having a mobility at the operating temperature of at least  $2 \text{ cm.}^2/\text{volt-sec.}$

The invention relates to an electric incandescent lamp which employs a filament of a material having a specific selective light emission in the visible part of the spectrum.

It has been proposed repeatedly to improve the luminous efficiency of thermal radiators by using filaments with selective radiation properties. Such a filament must have emission capacity in the visible range approaching unity but for all the other wavelengths, in particular in the near infrared region, it should be very small.

As is known, for example, in incandescent lamps employing a filament of tungsten, the adverse energy losses, which may be approximately 97%, mainly consist of infrared radiation. This is due to the fact that tungsten has an emission capacity which, in the infrared region, is only slightly lower than in the visible region.

As selective radiators only non-metallic, non-conductive or semi-conductive substances, for example, oxidic materials having high melting points, in particular ceramic materials which may be colored in addition are actually known so far. Such radiators require special lamp constructions; in general, a ballast impedance must be used. For starting such lamps in operation often heat has to be applied to the filament externally, for example, in the form of a gas-discharge. As a result of these and other difficulties lamps with such radiators have not found universal acceptance. On the other hand, attempts have been made to increase the efficiency of tungsten incandescent lamps by higher operating temperatures, for example, by using transport reactions as is the case in the tungsten-iodine-cycle.

The object of the invention is to use compounds with metallic conductivity which, in contrast with the known metals with high melting points, have a specific selectivity as to their light emission at high temperatures.

In the investigation which has resulted in the invention it has been found that such compounds must have certain properties with respect to the concentration of the free charge-carriers and the mobility of such carriers.

As a result of the absorption of the free charge carriers, the said compounds, already in layers having a thickness of approximately  $1\mu$  will not be transparent throughout the entire visible region and the infrared region of the spectrum. In this condition the emission capacity is equal to  $I-R$ . In the ideal case it is endeavoured to obtain a reflection of unity in the infrared region to make the emission equal to 0, while on the other hand in the visible region the reflection should be small and as a result the emission capacity would have to be large.

The reflection R can be expressed by certain parameters of the material. The theory of the optical constants of free

2

carriers gives the known relations for the real and the imaginary part of the coefficient of reflection  $n^* = n - iK$ :

$$n^2 - K^2 = \epsilon_g = \frac{Ne^2}{m^* \epsilon_0 (\omega^2 + \gamma^2)}$$

and

$$2nK\omega = \frac{\gamma Ne^2}{m^* \epsilon_0 (\omega^2 + \gamma^2)}$$

K is related to the absorption coefficient  $\alpha$  of the medium by the relation  $\alpha = 4\pi K/\lambda$ .

In the above relation:

$n$ —Coefficient of refraction of the medium

$\epsilon_g$ —Dielectric constant of the medium in the absence of free carriers

$N$ —Concentration of charge carriers

$e$ —Elementary charge

$m^*$ —Effective mass of the charge carriers, which is defined by the relation  $F = m^* dv/dt$ , where F is the external force, for example, of an electric field, and v the velocity of the carriers

$\epsilon_0$ —Dielectric constant of the vacuum

$\omega$ —Angular frequency of the light

$\gamma$ —Damping constant which is equal to  $e/\mu m^*$ , where  $\mu$  is the mobility of the carriers.

From these equations  $n$  and  $K$ , and therefrom the reflection according to

$$R = \frac{(n-1)^2 + K^2}{(n-1)^2 + K^2}$$

can be calculated for all wavelengths. A reflection curve is then obtained as is shown in FIG. 1. Starting at short waves, the reflection traverses at least one minimum and then rapidly rises to high values. It is required that the transition from low to maximum reflection of a selective radiator be effected within a small wavelength interval. In a thermal selective radiator the said transition should lie on the boundary between the visible region and the infrared region, i.e., at approximately  $0.7 \mu\text{m}$  which corresponds to an angular frequency of  $2.7 \times 10^{15} \text{ sec.}^{-1}$ . This frequency is fixed by the condition  $n^2 - K^2 = 0$  and

$$\omega_0 = \frac{Ne^2}{\epsilon_0 \epsilon_g m^*} - \gamma^2$$

is obtained.

When  $\gamma$  is negligibly small, the concentration N of carriers required for the desired angular frequency can be evaluated from this formula to be at least  $2.2 \times 10^{22} \text{ cm.}^{-3}$ . In this evaluation it is assumed that  $\epsilon_g$  is approximately 10 and that the effective mass  $m^*$  is equal to the mass of the free electron. Since the effective masses of charge carriers are generally smaller than those of the free electron, the said concentration of carriers must be considered to be the upper limit.

In experiments it has further been found that the concentration of the free charge carriers must be at least  $2 \times 10^{21} \text{ cm.}^{-3}$  and the mobility of the carriers at the operating temperature at least  $2 \text{ cm.}^2/\text{volt-sec.}$

It has now been found that the hexaborides of the rare earths and alkaline earth metals, particularly, readily meet the said requirements. This appears from the following table and the figures.

| Hexaboride Compound    | Concentration of the charge carriers per $\text{cm.}^{-3}$ | Mobility $\text{cm.}^2/\text{volt-sec.}$ | Reflection side in microns ( $\mu\text{m}$ ) |
|------------------------|------------------------------------------------------------|------------------------------------------|----------------------------------------------|
| LaB <sub>6</sub> ----- | $1.4 \times 10^{22}$                                       | 32                                       | 0.65                                         |
| CeB <sub>6</sub> ----- | $1.5 \times 10^{22}$                                       | 15                                       | 0.65                                         |
| PrB <sub>6</sub> ----- | $1.3 \times 10^{22}$                                       | 22                                       | 0.65                                         |
| NdB <sub>6</sub> ----- | $0.9 \times 10^{22}$                                       | 25                                       | 0.65                                         |
| YbB <sub>6</sub> ----- | $0.9 \times 10^{21}$                                       | 76                                       | 1.5                                          |

The invention will be described with reference to the accompanying drawing in which FIGS. 1, 2, 3 and 4 are curves showing the reflection of various materials as a function of wave-lengths and FIG. 5 shows a lamp according to the invention.

FIGURES 1, 2 and 3 show the reflection of  $\text{NdB}_6$ ,  $\text{PrB}_6$  and  $\text{CeB}_6$  as a function of the wavelength. In these cases the variation of the reflection shows great resemblance. In the direction from short to longer waves at least one minimum at  $0.6 \mu\text{m}$  is traversed, after which a steep ascent of the reflection follows.

FIG. 4 shows the reflection curve of  $\text{LaB}_6$  and  $\text{YbB}_6$ . Whereas the  $\text{LaB}_6$  behaves as the other hexaborides, the reflection side of  $\text{YbB}_6$  lies at approximately  $1.5 \mu\text{m}$ . The cause hereof must be considered to be the considerably lower charge concentration of the  $\text{YbB}_6$  (see the table).

Alternatively mixtures of the said compounds may be used. The reflection side may then be shifted continuously, for example, between the curves of  $\text{LaB}_6$  and  $\text{YbB}_6$  shown in FIG. 4.

The filaments can simply be manufactured ceramically, while it is also possible to borinate a coiled wire of, for example, lanthanum in known manner.

Thus, FIG. 5 shows an incandescent lamp employing a filament of  $\text{LaB}_6$  in an envelope 2 containing iodine vapor.

The vaporization or dissociation of the hexaborides during burning can be prevented to a great extent by using a cycle, for example, by using a volatile boro-halogen compound, for example,  $\text{BF}_3$ ,  $\text{BCl}_3$ , so at least the most volatile component of the compound is transported back to the filament during burning by means of a chemical transport reaction. The filaments which according to the invention comprise a selectively radiating body need no ballast impedance or additional means for heating the filament.

What is claimed is:

- 4
1. An incandescent lamp employing a selectively radiating filament emitting principally visible radiation at a given operating temperature and consisting of a material having a concentration of charge carriers between  $2 \times 10^{21}$  and  $2 \times 10^{22}$  per  $\text{cm}^3$ , and the mobility of the charge carriers at the operating temperature of the radiator being at least  $2 \text{ cm}^2/\text{volt}\cdot\text{sec.}$ , said filament consisting of a hexaboride of an element selected from the group consisting of lanthanum and the rare earth metals.
  - 10 2. An incandescent lamp as claimed in claim 1 including means to return to the filament at least the most volatile component of the compound of which the filament exists by means of a chemical transport reaction.
  - 15 3. An incandescent lamp as claimed in claim 1 in which the filament consists of  $\text{LaB}_6$ .
  4. An incandescent lamp as claimed in claim 1 in which the filament consists of  $\text{YbB}_6$ .
  5. An incandescent lamp as claimed in claim 1 in which the filament consists of  $\text{NdB}_6$ .
  - 20 6. An incandescent lamp as claimed in claim 1 in which the filament consists of  $\text{PrB}_6$ .
  7. An incandescent lamp as claimed in claim 1 in which the filament consists of  $\text{CeB}_6$ .
  - 25 8. An incandescent lamp as claimed in claim 2 in which the means for returning the volatile component to the filament is a borohalogen compound.

#### References Cited

#### UNITED STATES PATENTS

- |    |           |        |                        |           |
|----|-----------|--------|------------------------|-----------|
| 30 | 3,132,278 | 5/1964 | Collins et al. -----   | 313—222 X |
|    | 3,134,924 | 5/1964 | Henderson et al. ----- | 313—218 X |
|    | 3,334,261 | 8/1967 | Butler et al. -----    | 313—227 X |

JAMES W. LAWRENCE, Primary Examiner.

35 P. C. DEMEO, Assistant Examiner.